

## UNITED STATES PATENT OFFICE

2,369,705

## GREASE

Fred E. Woodward and Jerome W. Arkis,  
Davenport, IowaNo Drawing. Application July 8, 1942,  
Serial No. 450,184

2 Claims. (Cl. 252—37)

(Granted under the act of March 3, 1883, as  
amended April 30, 1928; 370 O. G. 757)

The invention described herein may be manufactured and used by or for the Government for governmental purposes without the payment to us of any royalty thereon.

The present invention relates to lubricants and more particularly to an improved grease, stabilized against deterioration in the presence of oxygen.

Prior art greases heretofore employed in the recoil mechanisms of modern artillery pieces, rapidly break down when subjected to an oxygen-containing atmosphere, particularly in the presence of copper or alloys thereof. With such prior art greases, copper or an alloy thereof appears to act as a decomposition accelerator or catalyst, greatly increasing the rate of breakdown of the grease in the presence of oxygen. Thus it has been found, using the Norma-Hoffmann accelerated stability test for lubricating greases (A. S. T. M. Preprint No. 94, 1938), that the induction period of prior aluminum base recoil greases drops from some 960+ hours, when the test is carried out in glass dishes without a catalyst, to perhaps 48 hours or lower when the test is performed in the presence of a catalyst comprising naval brass. In view of the fact that recoil mechanisms usually contain copper or alloys thereof such as brass, it is apparent that an improved stabilizer is required for recoil greases so that such greases may be made proof against oxidative deterioration in the presence of copper-containing metals.

The object of the present invention is to provide a grease characterized by increased stability to oxygen in the presence of copper or copper alloys such as brass.

A further object is to provide a means for increasing the oxygen induction period for aluminum base recoil greases when tested by the Norma-Hoffmann accelerated stability test in the presence of copper containing catalysts.

Another object is to provide a method of stabilizing recoil greases of all types, against oxidative deterioration in the presence of copper or copper containing metals.

Still another object is the provision of a new and improved grease stabilizer which greatly increases the stability of greases to the destructive effect of oxygen in the presence of a copper-containing catalyst, which stabilizer does not impair the other desirable properties of the grease.

Other objects and advantages of the present

invention will appear as the invention is herein-after more particularly described.

We have found that the foregoing objects may be accomplished in accordance with the present invention, one aspect of which involves the incorporation in the recoil grease, of a small percentage of a stabilizer selected from the group consisting of:

- 10 (a) Aryl-substituted naphthyl amines, such as phenyl beta naphthyl amine;
- (b) Aryl-substituted arylene diamines, such as diphenyl para phenylene diamine; or
- (c) Alkoxy diaryl amines, such as dipara-methoxydiphenylamine.

15 The foregoing stabilizers may be used singly, or in combination with each other, or in combination with other compounds, as desired.

In carrying out a preferred embodiment of the present invention, the herein disclosed stabilizers, either singly or in combination, are incorporated at any suitable step in the compounding of the grease. Thus, for example, the improved stabilized grease of the present invention may be compounded by first incorporating a conventional grease-base soap (for example, aluminum

20 stearate, oleate and/or palmitate) in a suitable grease-base oil. After the soap and oil have been suitably mixed, a small percentage, for example 1% (based on the weight of the soap and oil) of the inhibitor is added to the grease-base. In some instances it may also be desirable to incorporate a small percentage of a free fatty acid, such as stearic acid, in order to overcome any tendency of the ultimate grease, to bleed.

25 After the components have been thoroughly mixed, the grease is maintained at an elevated temperature in order to permit the escape of any occluded air. When the air has been completely removed, the grease is allowed to chill very slowly, thereby insuring a grease having a proper jell and consistency.

In order more clearly to disclose the nature of the present invention, a preferred embodiment 30 thereof will hereinafter be described. In this example, phenyl beta naphthyl amine will be employed as the specific stabilizer. It should be clearly understood, however, that this is done solely by way of example and is not to be construed as a limitation upon the spirit and scope 35 of the appended claims, inasmuch as any of the foregoing stabilizers may be substituted for the

rticular compound given in the illustrative example:

**EXAMPLE**

A suitable grease-base oil such as heavy recoil is weighed out in an amount sufficient to provide 83.8% by weight of the ultimate grease. hereafter 15% of a metal soap such as commercial "aluminum stearate" (usually a mixture of the stearate, oleate and palmitate) is then added to the oil and the mixture thoroughly agitated in the cold in order to wet the soap with the oil. Thereafter the oil and soap may be permitted to stand. However, if preferred, the mixture may be heated immediately to approximately 325-359° F., with constant agitation, in order to melt the soap. When the soap has been completely melted and thoroughly incorporated in the oil, 1% of phenyl beta-naphthylamine is stirred into the grease. Preferably there is also incorporated at this time approximately 0.2% of free fatty acid, such as stearic acid, the particular amount selected being sufficient to insure that the ultimate grease will not be alkaline in reaction.

The agitation of the mixture is continued for about half an hour after which the material is drawn or run into shallow containers which are then placed in an oven heated to approximately 50°. The containers are allowed to remain in the oven for approximately 24 hours in order to allow occluded air to escape. The initial temperature of 350° F. may be very gradually reduced over the twenty-four hour period, or the grease may be held at a constant temperature for the initial twenty-four hour period and thereafter permitted to chill very slowly. The latter method of cooling is usually preferable inasmuch as it insures a grease which has a proper jel and which also will not show any tendency to bleed.

In some instances, it may be desirable to add other stabilizers in addition to the phenyl beta-naphthylamine employed in the foregoing example. Thus for example, the stabilizer may consist of two parts by weight phenyl beta-naphthylamine, one part by weight diparamethoxydiphenylamine and one part of diphenylparaphenylene diamine, this mixture being employed in the grease to the extent of 1% by weight. In other instances it may be desirable to use the various stabilizers individually or in various proportions. Although we have discovered that the employment of a stabilizer comprising substantially one per cent (1%) by weight of the total weight of the grease provides optimum antioxidant performance from the economic standpoint it will be apparent that other percentages of stabilizer may also be employed, the antioxidant effect thereof being dependent to a certain extent upon the quantity or proportion used.

In order to establish the stability of greases prepared in accordance with the present invention, experiments were conducted using the Norma-Hoffmann accelerated stability test for lubricating greases. This procedure included the loading of various greases, prepared under identical conditions, in a Norma-Hoffmann bomb. Each dish of the bomb contained a naval brass catalyst having a surface area of 0.756 square inch. The subsequent details of the tests were similar to those set forth in the A. S. T. M. Preprint mentioned above. The results are indicated in the table.

**Table**

|    | Inhibitor and content | Induction period (I. P.) | Pressure drop during I. P./100 hrs.(P.D.) | Condition of grease after oxidation | Condition of catalyst after oxidation |
|----|-----------------------|--------------------------|-------------------------------------------|-------------------------------------|---------------------------------------|
| 5  | A 1 (1%)              | 189                      | 4.8                                       | Semi-liquid, rancid.                | Green coating.                        |
| 10 | B 2 (1%)              | 384                      | 4.75                                      | Liquid, rancid                      | Slight corrosion.                     |
| 15 | B 3 (0.50%)           |                          |                                           | Black semi-solid, rancid.           | Green coating.                        |
| 20 | C 3 (0.25%)           | 413                      | 4.44                                      |                                     |                                       |
| 25 | D 4 (0.25%)           |                          |                                           |                                     |                                       |

<sup>1</sup> A—phenyl alpha naphthylamine.

<sup>2</sup> B—phenyl beta naphthylamine.

<sup>3</sup> C—diparamethoxydiphenylamine.

<sup>4</sup> D—diphenyl para phenylene diamine.

As will be apparent from the induction periods noted in the foregoing table, a grease-containing phenyl beta naphthylamine is substantially more stable under the conditions of the test than a grease containing the alpha position isomer (384 compared with 189). Further improvement was noted when the other inhibitors were incorporated along with the phenyl beta naphthylamine, as indicated by the last example in the table (I. P.=413). The grease represented by sample "A" is, in turn, far more stable than the same grease without the phenyl alpha naphthylamine, as indicated by the fact that a similar grease containing no inhibitor will frequently show an induction period below 30, and greases containing the usual commercial "metal deactivators" do not show any measurably greater stability under the conditions of the test. It will thus be seen that the incorporation of a very small percentage of the improved stabilizers of the present invention results in an entirely unexpected (and indeed, inexplicable) enhancement in stability of greases under the conditions of the Norma-Hoffmann test, when carried out in the presence of a copper-containing metal.

In the foregoing detailed description it will be apparent to those skilled in the art that many variations may be made without departing from the spirit and scope of the present invention. Thus for example, although the invention has been illustrated by particular reference to the phenyl-substituted beta-naphthylamines, the other aryl amino stabilizers hereinbefore described may be employed where desired, the particular compound selected being determined in part by the availability of the compound in question. Many other variations will be apparent to those skilled in the art. We therefore intend to be restricted only in accordance with the following patent claims.

We claim:

1. A grease comprising an oil, a metal soap, and a stabilizer consisting substantially of a mixture of about 25% diparamethoxydiphenylamine, about 25% diphenylparaphenylene diamine and about 50% phenyl beta naphthylamine.
2. A grease comprising a metal soap, an oil, and an antioxidant stabilizer comprising substantially one per cent (1%) by weight of said grease, said stabilizer comprising substantially a mixture of about 25% diparamethoxydiphenylamine, about 25% diphenylparaphenylene diamine and about 50% phenyl beta naphthylamine, and wherein said soap comprises an aluminum salt of a long chain fatty acid.

FRED E. WOODWARD.  
JEROME W. ARKIS.

## CERTIFICATE OF CORRECTION.

Patent No. 2,369,705.

February 20, 1945.

FRED E. WOODWARD, ET AL.

It is hereby certified that error appears in the printed specification of the above numbered patent requiring correction as follows: Page 2, first column, line 15, for "325-359° F." read --325-350° F.--; and that the said Letters Patent should be read with this correction therein that the same may conform to the record of the case in the Patent Office.

Signed and sealed this 19th day of June, A. D. 1945.

Leslie Frazer

(Seal)

Acting Commissioner of Patents.